# EUROPEAN PATENT SPECIFICATION

(11) **EP 1 244 819 B1**
(45) Date of publication and mention of the grant of the patent: **10.08.2005**
(21) Application number: 00984732.8
(22) Date of filing: 15.12.2000
(51) Int. Cl.: C22F 1/04, C22F 1/047, C21D 9/573

(54) **METHOD OF QUENCHING AN ALLOY SHEET TO MINIMIZE DISTORTION**
VERFAHEN ZUM ABSCHRECKEN EINES LEGIERUNGSBLECHES ZUR MINIMIERUNG VON VERZIEHUNG
PROCEDE DE TREMPE DE FEUILLE D'ALLIAGE POUR MINIMISER LA DEFORMATION

(30) Priority: 17.12.1999 US 467306
(43) Date of publication of application: 02.10.2002
(73) Proprietor: ALCAN INTERNATIONAL LIMITED, Montreal Quebec H3A 3G2 (CA)
(72) Inventor: GUPTA, Alok, Kumar, Kingston, Ontario K7M 1F2 (CA); LAGACE, Helene, P., Kingston, Ontario K7L 4V4 (CA); JEFFREY, Paul, W., Kingston, Ontario K7M 5A6 (CA); URBANEK, Jaroslav, Anna Maria, FL 34216 (US); DAVENPORT, Christopher John, Bilton, Rugby, Warwickshire CV22 7RS (GB)
(74) Representative: Gaunt, Robert John
(86) International application number: PCT/CA2000/001522
(87) International publication number: WO 2001/044532

(56) References cited:
- EP-A- 0 949 348
- WO-A-98/42885
- DE-A- 1 508 432
- US-A- 4 610 735

## Description

### TECHNICAL FIELD

The present invention relates to methods of quenching heat-treatable aluminum alloy sheet from solutionizing temperatures to fabricate alloy sheet in either the T4 or T4P tempers, which are the conditions in which such sheet articles are normally supplied to automobile manufactures and other users. More particularly, the invention relates to methods of this kind intended to minimize distortions of the sheet articles caused by thermal stress generated during quenching.

### BACKGROUND ART

Manufacturers of aluminum alloy sheet articles are faced with the challenge of providing thin-gauge sheet materials that have both good formability in the supplied temper and high strength after a part has been formed from the sheet and paint-cured. The automobile industry, in particular, demands such products for use as the raw material for producing body panels or structural members of reduced weight in the ongoing quest for improved vehicle economy and fuel efficiency.

It has become common place to make use of heat-treatable AA (Aluminum Association) 6000 series, or some AA2000 series, aluminum alloys for the production of such sheet articles. Heat-treatable alloys are generally those containing soluble alloying constituents in amounts that exceed their room temperature solubility limits. Such alloys may develop enhanced properties upon being subjected to working and/or heating, followed by a quenching step. These alloys usually contain hardening elements (e.g. magnesium, silicon and/or copper) to provide hardening during aging, and other elements, like Fe, Mn and possibly Cr, to control the formability and grain size. Such alloys are generally direct chill (DC) or continuously cast and homogenized above the solvus temperature (which is defined as the temperature above which all the soluble particles, e.g. Mg₂Si, Al_{w}CuₓMg_{y}Si_{z} (referred to as Q or Q-phase), and other particles depending on the alloy composition, become unstable and dissolve in the aluminum matrix), in order to dissolve the soluble particles present in the as-cast ingot or continuous strip, and to improve hot ductility for subsequent thermo-mechanical processing steps. The homogenized ingot is hot- and cold-rolled to the final gauge with or without an intermediate annealing step. The final gauge sheet material is then solutionized above the solvus temperature (usually in the range of 480 to 580°C) to dissolve the soluble particles that are formed during the hot- and cold-rolling, and then quenched to obtain the desired T4 or T4P temper.

The quenching process is one of the most critical steps in producing an acceptable sheet material in the supplied temper. The material is considered highly undesirable if it contains coarse grain boundary particles since they affect the mechanical properties of the sheet, such as its bendability, and to some extent the hardening response during the paint cure. Therefore, it is essential that the sheet material be rapidly quenched from the solutionizing temperature to avoid precipitation of the harmful secondary phase particles on the grain boundaries, and occasionally within the matrix, and to obtain the best combination of formability in the supplied temper and hardening response during the paint cure.

Unfortunately, rapid quenching from solutionizing temperatures can result in permanent distortion of the sheet article, particularly for thin gauge products. When such distortion occurs, the sheet must be flattened mechanically more than usual by stretching and/or bending to remove the distortions. This decreases the formability of the material due to the cold working that is introduced during the stretching operation. It would therefore be advantageous to avoid such distortion during quenching procedures, and this goal has already been given consideration in the prior art. However, steps taken to avoid or minimize distortion can adversely affect the intended advantages of the quenching operation, or can introduce costly and inconvenient steps into the quenching process.

U.S. Patent No. 4,784,921, which issued on November 15, 1988 to M. E. Hyland, et al., discloses a method of producing aluminum sheet materials suitable for vehicle panels. The method involves a solution heat treatment followed by rapid quenching at a rate of at least 10°F/sec (preferably at least 300°F/sec) from the solutionizing temperature by means of liquid cooling. After the sheet has reached a temperature of 350°F or less, air-cooling may be employed to ambient temperature.

Similarly, U.S. Patent No. 5,061,327, which issued on October 29, 1991 to D. K. Denzer, teaches of a method preferably involving a cold water quench directly from the solutionizing temperature. The preferred method involves sheet alloy quenching in water to approximately 93°C at a rate greater than or equal to 56°C/sec, followed by air cooling to ambient temperature.

PCT publication WO 98/42885 of October 1^{st}, 1998 filed in the name of Aluminum Company of America discloses a process for the manufacture of metal alloy sheet without distortion wherein a controllably variable liquid quenching means is used to control the time at which an alloy strip remains above a critical temperature (the so-called Leidenfrost temperature - i.e. the temperature above which a vapor layer is present between the sheet surface and the liquid cooling film). It is said that the liquid quench cools the metal through the critical temperature at a rate that can be controllably varied for each metal alloy composition and can increase or at least maintain the strength potential of the alloy without physical distortion. However, this reference links the cooling to variables that have nothing to do with the identity and characteristics of the material being cooled. The publication states that the Leidenfrost temperature is functionally and operatively related to the specific spray orifice used for the cooling liquid, the flow rate, the physical and chemical properties of the liquid, and the pressure used to apply the liquid. It is therefore difficult to achieve the best results for any particular alloy without carrying out complicated adjustments. Also, while the material may have a gas layer separating the hot material from the cooling liquid, this gas layer is created by evaporation of the cooling liquid, which requires the extraction of heat of vaporization from the material, thus providing a significantly higher cooling rate than would be the case if a change of state from a liquid to a gas were not involved.

The document US-A-4 610 735 discloses a method for minimizing deformation during rapid cooling of flat metallurigcal products such as sheets, strips, flattened portions, wide sections and the like. The method comprises rapidly cooling the product by means of a fluid (or mixtures of fluids) at temperature TF, comprising at least one vaporizable liquid, with modulation in a direction perpendicular to the direction of advance of the product, so as to impart different cooling speeds to the edges and the axis (case I) or to one edge and the other (case II). The technique may be completed by careful masking of the cooling in the zone for the rapid cooling action, or by controlled precooling prior to said rapid cooling. The method makes it possible to obtain the rapid cooling which is necessary e.g. in quenching operations, while at the same time minimizing the deformations or the internal stress level of flat products.

Consequently, the inventors of the present invention have found that methods involving liquid quenching from solution temperatures are difficult to control in a way that enables thermal distortion to be minimized while retaining good formability in the as-supplied tempers and high strength after the part has been formed and paint cured.

### DISCLOSURE OF THE INVENTION

An object of the present invention is to provide a method of quenching a sheet article of solution heat treated aluminum alloy in a way that minimizes or avoids distortion of the article, while also avoiding undue precipitation of second phase particles from the metal.

Another object of the invention is to provide such a method that can be carried out in a practical and relatively inexpensive manner.

Another object of the invention is to provide a method of producing an article made of heat-treatable alloy in T4 or T4P temper by casting, homogenizing, rolling, and heat treating, while employing a solutionizing and quenching step that avoids undue distortion and particle precipitation.

The invention is defined in claims 1 and 13.

The gas cooling step has the practical effect of lowering the liquid-quench start-temperature for the subsequent liquid cooling step that is carried out at a high rate of cooling and that consequently generates high thermal stresses. At the lower liquid-quench start-temperature, the alloy has an increased yield strength compared to that at the solutionizing temperature, and is therefore better able to resist thermal deformation.

The initial cooling of the article in the gas (referred to as slow cooling) may be accomplished by using heated air as the cooling medium in one or more successive zones of a heat treatment apparatus through which the article is passed immediately following the heating zone of a continuous heat treatment furnace. The heated air in the cooling zone is preferably directed onto one or both of the surfaces of the sheet article from suitable gas nozzles. The temperature within the cooling zones may be set at different (progressively lower) temperatures to successively increase the quenching rate in approximate proportion to the increase of yield strength of the metal that occurs with decreasing temperature. In this way, very low quenching stresses are initially introduced while the metal yield strength is low.

The quenching steps of the invention are acceptable metallurgically because no detrimental precipitation takes place above the upper critical temperature of the precipitation range. Therefore, the slow quenching at high temperature does not affect the eventual metallurgical structure of the alloy sheet product. Once the upper critical temperature has been reached, rapid quenching may be carried out to avoid precipitation without causing thermal distortion. The additional cooling to a temperature below the lower critical temperature (e.g. ambient or room temperature), if required at all, is then preferably carried out in a gas, such as air, but the manner of cooling is not critical, so liquid cooling could alternatively be employed for this step, or the metal could merely be allowed to stand and cool naturally.

The invention is particularly applicable to the treatment of AA6000 series aluminum alloys. In such cases, the upper critical temperature is about 450°C (but may be as low as about 400°C) and the lower critical temperature is about 325°C (but may be as low as about 300°C), and the step of cooling the sheet article with a gas from the solutionizing temperature to the upper critical temperature (gas cooling) is carried out at a rate of between 10°C/second and 200°C/second, and preferably at approximately 20°C/second. The further cooling from the upper critical temperature to the lower critical temperature (liquid cooling) is conducted at a rate of between 200°C/second and 2000°C/second, and preferably between 200°C/second and 450°C/second.

The present invention provides an efficient and productive method of minimizing thermal distortion during cooling of a sheet alloy from the solution heat treatment temperature. The method has the considerable economic advantage that it may be carried out in conventional quenching equipment (e.g. a continuous heat treatment line), without undue difficulty and normally without requiring expensive modifications.

The present invention is applicable to all heat treatable alloys that are subjected to solutionizing and quenching during processing, e.g. aluminum alloys of the AA6000 series, AA2000 series, AA7000 series and Al-Li type alloys. Although the critical temperature range (upper critical temperature and lower critical temperature) and the desired cooling rates may be different for different alloys, the appropriate ranges and cooling rates for each alloy may be determined by simple experimentation, e.g. by direct observation of the microstructures of metal samples rapidly down-quenched and held at different temperatures (heat soak temperatures) below their solutionizing temperatures and then rapidly water-quenched to ambient. The direct observation can be achieved by means of a transmission electron microscope. Observation of the first evidence of extensive precipitation of Q-phase particles at a particular soak temperature determines the upper critical temperature, and evidence of no further substantial precipitation of such particles determines the lower critical temperature.

The maximum rate of cooling to be used above the upper critical temperature (gas cooling) may also be determined by experimentation, e.g. by observing degrees of distortion (if any) in samples cooled at different rates in the gas cooling stage, and deciding which degrees of distortion are to be avoided.

It should be realized that the term "sheet" as used herein refers to a generally flat (planar) article, often (but not necessarily) of indefinite length. The thickness of such articles is not particularly relevant, although automotive sheet articles (e.g. of AA6111 alloy) subjected to solutionizing and quenching normally have a thickness of 2.3 mm or less, typically 0.8 to 2.0 mm. However, the term "sheet" as used herein is intended to includes a product often referred to as "plate" (generally taken to mean a rolled product that is rectangular in cross-section having a thickness not less than 0.250 inch (6.35 mm) with sheared edges). While the present invention is primarily concerned with planar articles, such as metal sheet, the method may also be applied to shaped products, such as extrusions, in which distortion is a factor.

### BRIEF DESCRIPTION OF THE DRAWINGS

Fig. 1 is a graph showing how yield strength (YS) of an alloy (in this case alloy AA6111) declines as the temperature of the alloy increases and, in particular, how the YS declines rapidly in the upper temperature range (e.g. above 450°C);
Fig. 2 is a graphical illustration of various quenching methods for AA6111 aluminum alloy according to the prior art and preferred embodiments of the present invention;
Fig. 3 is a schematic diagram showing a simplified cross-section of a part of a heat treatment apparatus suitable for carrying out one preferred form of the present invention; and
Figs. 4 and 5 are graphs representing typical temperature profiles of sheet articles passing through heating and cooling zones of the heat treatment apparatus. The cooling profile shown is in accordance with the present invention.

### BEST MODES FOR CARRYING OUT THE INVENTION

The present invention provides a method for minimizing or eliminating permanent distortion of alloy sheet or other heat-treatable materials caused by the thermal stresses associated with quenching practices following solution heat treatments, while retaining the desirable effects of such solutionizing to the greatest possible extent.

Rapid quenching of heat treatable alloys is required in order to maximize the formability in the as-supplied (to the user) temper while obtaining high strength, durability and good corrosion resistance in the final product to meet the strict requirements of the automotive industry and other users. However, the inventors of the present invention have realized that such rapid quenching is necessary only within the range of temperatures in which second phase precipitation may occur. At temperatures above this range, a slower rate of cooling may be adopted without significantly affecting the metallurgical structure of the metal, and a rate of cooling may be chosen at which the yield strength of the metal remains high enough to resist thermal stresses generated by the cooling procedure, thus minimizing or eliminating permanent deformation of the sheet product. Such deformation is, in fact, only likely at high temperatures where the yield strength of the alloy is extremely low compared to the yield strength at ambient temperature. For most heat-treatable aluminum alloys, once the temperature has been reduced to the precipitation range, high rates of cooling may be employed without causing deformation because the yield strength of the alloy at these temperatures has increased significantly compared to the yield strength at the solutionizing temperature.

Accordingly, the present invention divides the cooling operation from the solutionizing temperature into two or more distinct steps. The first step involves a slow rate of cooling (achieved by gas cooling in a heated gas) from the solutionizing temperature to the upper critical temperature below which precipitation may occur, and a second step involves rapid cooling (achieved by liquid quenching, or mixed liquid and gas quenching) right through the precipitation range between the upper and lower critical temperatures. The nature of the further cooling (if any) carried out below the lower critical temperature of the precipitation range is less critical and may be carried out at any desired rate using either liquid cooling or gas cooling, although gas cooling employing air is preferred. At these lower temperatures the yield strength of the alloy is high enough to resist thermal deformation without allowing precipitation of detrimental particles on the grain boundaries.

The alloy thus obtained is generally aged, following quenching, to obtain the desired T4 or T4P tempers.

Fig. 1 is a graph showing how the yield strength (YS) of a typical AA6000 series alloy (specifically AA6111) falls as the temperature of the alloy is raised. The vertical axis (ordinate) shows the yield stress at a particular temperature expressed as a percentage of the room temperature yield stress (R.TempYS). It will be seen that the yield stress falls rapidly to zero as temperatures increase from about 450 to 600°C. Solutionizing often takes place at temperatures up to about 600°C, so the metal is very susceptible to deformation at these temperatures. On the other hand, at a temperature of about 450°C, approximately 50% of the room temperature yield stress has been developed, so the material is quite deformation-resistant below this temperature. For AA6000 series alloys, this is generally the upper critical temperature of the precipitation range.

The present invention is described in particular as being a method of processing aluminum alloy sheets of the Aluminum Association AA6000 series aluminum alloys and some AA2000, AA7000 and Al-Li alloys. However, it is fully contemplated that the methods of the present invention provide thermal mechanical processing procedures which can be beneficial to the working of a variety of heat-treatable alloys, including other categories of aluminum alloy, provided the upper end of the temperature range at which significant precipitation may take place is sufficiently low that, for the alloy in question, rapid quenching may be initiated from that temperature without significant distortion of the alloy sheet product. That is to say, at the upper critical temperature of the alloy in question, the yield strength of the alloy should be high enough to resist thermal stresses caused by rapid quenching. At temperatures above the critical temperature, the cooling rate is slowed to allow the yield strength of the alloy to increase before significant thermal stresses are imposed.

Fig. 2 illustrates temperature-time correlation curves for AA6111 alloy sheet product. The figure includes regions A, B and C depicting temperature ranges of importance to the present invention. Region A is the temperature range between the solutionizing temperature (Tₛₒₗ) and the upper critical temperature (Tᵤₚₚₑᵣ) below which precipitation may commence. Region B represents the precipitation range (critical range) in which secondary phase precipitation may take place if the time and temperature conditions are appropriate. Region C is the range of temperatures below T_{lower}, the temperature below which further secondary phase precipitation does not take place at any rate of cooling. It should be noted that these ranges in temperature are not absolute, and will vary for any given quenching method depending upon the physical properties of the subject alloy. The temperature ranges can, however, be determined experimentally for any given heat treatable alloy.

Three quenching procedures are illustrated in Fig. 2, namely Quench 1, Quench 2 and Quench 3. These procedures differ only prior to time "ts", i.e. the time from the termination of solutionizing at which the alloy temperature first reaches Tᵤₚₚₑᵣ. Following this time, the three procedures follow the same curve.

Quench 1 depicts a typical temperature gradient for quenching methods of the prior art, while Quench 2 and Quench 3 depict temperature gradients of the methods embodied by the present invention.

In accordance with common practices of the prior art, the quenching process is generally a single step process, which provides rapid cooling directly from the heat solutionizing temperature (Tₛₒₗ) through the critical precipitation temperature range. As illustrated in Fig. 2, the temperature gradient of Quench 1 is generally uniform through regions A and B. In contrast, Quench 2 and Quench 3 provide at least one preliminary step of slow cooling through region A before initiating the rapid cooling step through region B. The initial cooling of the sheet alloy within region A of Fig. 1 is conducted by the application of heated air in a manner such that thermal stress in most or all of the sheet alloy does not exceed the yield strength of the sheet. This slow cooling using heated air allows the temperature of the sheet alloy to approach the critical Tᵤₚₚₑᵣ temperature at a rate sufficiently slow to avoid high thermal stresses while allowing the development of properties of strength and stability sufficient to withstand the high thermal stresses generated at the onset of rapid quenching.

The rate of cooling and the temperature of the heated air required to produce this rate of cooling can be found empirically. Alternatively, the rate of cooling may be determined by applying a mathematical model that uses temperature, pressure, speed, product gauge and the heat transfer coefficient to calculate the optimum temperature of the heated air based on the temperature of the metal following the solutionizing treatment. The temperature of the cooling gas may be determined using the same mathematical model and varies with the peak metal temperature targeted. A typical range of gas temperatures suitable for the AA6111 alloy would be from 300 to 350°C.

The heated air may be applied in one or more successive zones of a continuous heat treatment apparatus to gradually cool the sheet alloy. Upon reaching Tᵤₚₚₑᵣ, rapid quenching using water or any other standard high heat capacity liquid (or mixture of gas and liquid), is initiated in further cooling zones to provide rapid cooling of the alloy sheet through a temperature range in which alloy precipitation would readily occur if the rate of cooling were sufficiently slow. At this stage of quenching, the yield strength of the sheet alloy has substantially increased from the yield strength at the solutionizing temperature. As such, the sheet alloy is capable of withstanding the stress of the quenching conducted through region B. In particular, the sheet alloy enters region B with sufficient strength to withstand the stresses from rapid cooling without suffering the consequence of permanent thermal distortion. The temperature of the cooling liquid used in this step may be much the same as the temperature of liquids used for conventional quenching steps. The temperature is generally between 18°C (ambient) and 30°C (warm).

Once cooled to a temperature in region C, which is below the range of precipitation (T_{lower}), the sheet is strong and no harmful precipitation occurs. The details of any further cooling that may be initiated are therefore less critical to the present invention. The temperature of the cooling medium used for this step may be controlled by the application of heat or cooling using heat exchangers. Typically, the temperature varies from 20°C to about 100°C.

The methods of the invention accordingly reduce distortion by exposing the sheet to a high quench rate only after the alloy is sufficiently cooled to withstand the associated stresses which accompany a rapid temperature drop. As a result, permanent distortion to the sheet alloy is minimized and often eliminated.

As noted, the first quenching step of the present invention occurs within region A of Fig. 2 where the sheet alloy is slowly cooled with air in one or more stages from the solutionizing temperature to a temperature just above the predetermined Tᵤₚₚₑᵣ temperature. The second quenching step occurs in region B and is indicative of the preferred rate of cooling through the critical temperature range. Table 1 further illustrates data on preferred and working temperatures associated with the present invention. It should be noted that the upper and lower range temperatures, as well as the working quenching rates, depend on the shape and position of the critical time curve (explained below), while preferred quenching rates are determined from the conditions which give the best combination of mechanical properties. Ideally, the closer the working temperatures come to the preferred temperature, the less thermal distortion expected in the sheet alloy product.

**Table 1.**

| Working and Preferred Quenching Rates for Air and Water Cooling Phases | | | | | |
|---|---|---|---|---|---|
| ALLOY | Range above Tᵤₚₚₑᵣ °C | Cooling Rate Range °C/s | | | |
| | | 1^{st} Step Cooling to Tᵤₚₚₑᵣ °C | | 2^{nd} Step Cooling below Tᵤₚₚₑᵣ °C | |
| | | Working | Preferred | Working | Preferred |
| AA6111 | ≥ 450 | 10-200 | ~ 20 (air cooling) | 200 - 2000 | 200 - 450 |
| AA6016 | ≥ 450 | 10 - 200 | ~ 20 (air cooling) | 200 - 2000 | 340 - 575 |

As illustrated in Fig. 2, the range of the critical time curve for AA6111 alloy is found to be within the range of 325°C to 450°C. The region above the Tᵤₚₚₑᵣ temperature (region A) represents the temperature range wherein slow cooling is preferred. This slow cooling step allows the sheet alloy to become stronger and thus be able to withstand the thermal stress of the subsequent aggressive quenching step. The conventional process as depicted as Quench 1, illustrates the onset an occasion of rapid cooling from the solutionizing temperature. The sheet alloy resulting from this treatment will suffer the effects of permanent distortion as a result of temperature gradients, induced by the rapid quench, exceeding the yield strength of the sheet alloy at or near the initial quenching temperature. Resulting sheet alloy must then be flattened mechanically by stretching and/or bending to remove the distortion. Such labor-intensive cold working efforts add to the cost of processing and decrease the formability of the material.

As further illustrated in Fig. 2, it is not until the temperature drops below Tᵤₚₚₑᵣ at time ts that rapid quenching must be initiated. Beginning at time ts, the time required to quench below T_{lower} directly determines the amount of precipitation which will occur. The figure shows a critical time curve S enclosing a shaded region E. At a temperature close to Tᵤₚₚₑᵣ, the driving force for precipitation of second phase particles is very small and nucleation and growth rates are slow thereby prolonging the start of the precipitation process. On the other hand, at temperatures around T_{lower} the driving force is very large and diffusion rates are too slow thereby impeding the onset of the precipitation process. Thus, precipitation rapidly occurs only at the nose N of the critical time curve C where a large driving force and high diffusion rates are present. The critical time curve S, as illustrated in Fig. 2, represents the beginning of this precipitation of second phase particles as a function of time and temperature. Thus, if the quenching curve crosses the shaded region E, secondary phase precipitation will take place to an undesirable extent. The properties of such a critical time curve, including the number, shape and position of the curve is largely dependent on alloy composition and the processing history of the alloy.

Therefore, an objective of the thermal mechanical processing of a sheet alloy in region B is to avoid the nose N of the critical curve C via rapid quenching and thus to eliminate the possibility of adverse effects caused by second phase precipitation. The time before the nose of the curve is called the incubation period, which is less than one second for AA6111. The precipitation process does not occur provided the time at temperature during quenching or aging is less than the incubation period or lies to the left of the critical curve.

Quench 2 of Fig. 2 employs a constant slow rate of cooling from the solutionizing temperature to Tᵤₚₚₑᵣ, the slope of the curve being gradual enough to avoid the generation of thermal stresses strong enough to exceed the yield strength of the alloy, and thus cause permanent deformation.

An alternative embodiment of the present invention is depicted in region A of Fig. 2 as Quench 3. In accordance with this embodiment a plurality of heated air phases are applied in the initial step of slow cooling to Tᵤₚₚₑᵣ to progressively increase the quenching rate in approximate proportion to the increase of yield strength with decreasing temperature. This can be accomplished by subjecting the alloy sheet to two or more heated air phases, operating at progressively lower air temperatures. In this manner, very low quenching stresses are initially introduced to the sheet alloy when the yield strength of the alloy is low.

Figure 3 is a simplified cross-section of part of a heat treatment apparatus suitable for carrying out a preferred form of the present invention. The apparatus 10 is in the form of a tunnel 11 through which the strip article 12 is drawn on a continuous basis. The apparatus is divided internally into a number of zones. A first zone 11A forms a last step of the solutionizing procedure. High temperature gas is introduced into the zone from nozzles 14 located in the top and bottom of the tunnel 11. The strip article passing through this zone is heated to the solutionizing temperature.

A second zone 11 B forms a region in which the temperature of the sheet article is cooled from the solutionizing temperature to Tᵤₚₚₑᵣ. Heated gas is injected into the zone through nozzles 15. As the strip article passes through this zone it may be cooled, for example, according to Quench 2 or Quench 3 of Fig. 2. Different temperature profiles in this zone can be obtained by varying the temperature of the gases passing through various nozzles in the zone.

The strip article then passes into a third zone 11C in which the article is quenched from Tᵤₚₚₑᵣ to T_{lower}. In the first part 16 of this zone, so-called "Coanda" nozzles 18 are provided to deliver a cooling liquid. The nozzles are positioned at an angle to the surface of the strip article 12 in the direction of sheet travel and mixes the cooling liquid (water) with air to reduce the droplet size. The smaller droplet size and angled positioning of the nozzle serve to improve the cooling efficiency. In this part of the zone 11C, the temperature of the strip article is above the Leidenfrost temperature and there is a vapour barrier between the liquid coolant (water) and the sheet surface. This arrangement provides more efficient cooling than just spraying cooling liquid directly onto the strip article. Once the temperature of the strip article passes through the Leidenfrost point, the vapour barrier disappears and conventional spray nozzles may be employed. This further cooling to T_{lower} is carried out in a second part 17 of the third zone 11C using conventional nozzles 20 oriented perpendicular to the surface of the strip article.

It should be noted here that, although the present invention makes use of liquid (or liquid/gas) cooling above the Leidenfrost temperature in the indicated embodiment, this is employed only below Tᵤₚₚₑᵣ and, in contrast, slow cooling by means of a gas is utilized above Tᵤₚₚₑᵣ. In this further respect, the present invention differs from the disclosure of WO 98/42885 (disclosed earlier) where there is no such slow gas cooling. WO 98/42885 commences with liquid cooling and follows with gas cooling, whereas the present invention does the opposite. Since the present invention starts the cooling with a gas, the heat transfer coefficient is inherently lower at this critical time than would be the case with liquid cooling as in WO 98/42885 (even taking into account the gas generation of the Leidenfrost effect because of the additional cooling effect due to a change of state of the cooling medium from liquid to gas).

In a fourth and final zone 11D, cooling below T_{lower} takes place by means of a gas introduced through nozzles 21.

Figures 4 and 5 are examples of temperature profiles of metal sheet articles positioned in heat treatment lines operated according to the present invention. These are graphs showing the predicted temperature with elapsed time of a point on the advancing metal strip article in solutionizing and cooling apparatus of the type shown in Fig. 3. Fig. 4 shows the predicted profile for light gauge sheet (1.00 mm), and Fig. 5 shows the profile for heavy gauge sheet (2.00 mm). The Figures show the rates of change of temperature of the metal in the various heating and cooling zones of the heat treatment line. In both cases, it will be seen that, following the peak solutionizing temperature, there is a slow cooling period A in a gas (heated air) preceding a rapid liquid (water) quench B, and then a further cooling period C to low temperature (post-quench cooling).

In practice, sheet material subjected to the heat treatments of Figs. 4 and 5 is found to be substantially free of thermal distortion while having good metallurgical properties suitable for use in the automotive industry.

For guidance in determining the upper and lower critical temperatures of different alloys, the following procedure is suggested. Samples of the alloy (e.g. aluminum alloy) are solutionized at 570°C for 2 minutes and then down-quenched and held in a second bath at different temperatures and times prior to water quenching to room temperature. The samples are examined in the transmission electron microscope to examine the quenched microstructures. The first evidence of extensive precipitation of Q phase observed is found, e.g. in a sample down-quenched to 400°C and held for 10 seconds. Similar microstructures are usually observed in samples down-quenched to different temperatures, e.g. 375°C and 350°C and held for 5 seconds at each temperature. The time taken for precipitation at particular temperatures may be noted, e.g. the time required at 300°C may be 30 seconds. A line joining the point where the first indication of precipitation is observed, on temperature-time axis, forms a TTT diagram for the formation of Q precipitates in the alloy in question. This diagram essentially provides the conditions for the formation of grain boundary Q precipitates in the alloy during the cool-down from the solutionizing temperature.

As a general point, it can be stated that, in accordance with the method of the present invention, detrimental alloy precipitation is avoided prior to rapid quenching. Accordingly, the present invention provides a sheet alloy of superior quality having preferred characteristics of workability, strength and durability. In addition, the present invention provides a method whereby thermal distortion is minimized and often eliminated. Therefore, the need for addition working after the performance of step-wise cooling of the present invention is obviated. Thus, there is provided a method to minimize distortion with improved overall efficiency. Accordingly, the sheet alloy produced by this method may have better strength and formability than sheet alloys of the prior art.

## Claims

1. A method of producing an article of solution heat treated aluminum alloy free of permanent thermal distortion, said alloy being capable of secondary phase precipitation during cooling only in a precipitation temperature range between an upper critical temperature in the range of 450°C to 400°C and a lower critical temperature in the range of 325°C to 300°C, said method comprising subjecting an article made of said heat-treatable aluminum alloy to a solution heat treatment at a solutionizing temperature above said upper critical temperature to dissolve soluble precipitates present in said alloy, quenching the article through said precipitation temperature range with a liquid or gas/liquid mixture at a rate of cooling between 200°C/sec and 2000°C/sec to avoid precipitation of said secondary phase particles, and optionally additionally cooling said article to a temperature below said lower critical temperature, **characterized in that** said article is cooled in a gas through an upper temperature range between said solutionizing temperature to said upper critical temperature at a rate of cooling within the range of 10°C/sec to 200°C/sec to avoid the generation of thermal stresses strong enough to exceed the yield strength of the alloy in said upper temperature range.

2. A method according to claim 1, **characterized in that** said cooling of said article below said lower critical temperature is carried out in a gas.

3. A method according to claim 1 or claim 2, **characterized in that** said cooling of said article below said lower critical temperature is carried out at a rate slower than said cooling through said precipitation range.

4. A method according to claim 1, claim 2 or claim 3, **characterized in that** the cooling of the article in the gas from said solutionizing temperature to the upper critical temperature is carried out in a single cooling zone.

5. A method according to claim 1, claim 2 or claim 3, **characterized in that** the cooling of the article in the gas from said solutionizing temperature to the upper critical temperature is carried out in a plurality of cooling zones.

6. A method according to claim 5, **characterized in that** the temperature of the gas in each successive cooling zone is progressively lower.

7. A method according to claim 6, **characterized in that** the lower temperatures are chosen to progressively increase the quenching rate in each zone in proportion to an increase of yield strength of the alloy in each zone.

8. A method according to any preceding claim, **characterized in that** said alloy of said sheet article is an AA6000 series aluminum alloy.

9. A method according to claim 8, **characterized in that** said step of cooling said sheet article from said solutionizing temperature to said upper critical temperature is conducted at a rate of approximately 20°C/sec.

10. A method according to claim 8 or claim 9, **characterized in that** said step of further cooling said sheet article from the upper critical temperature to the lower critical temperature is carried out at a rate of between 200°C/sec and 450°C/sec.

11. A method according to any preceding claim, **characterized in that** the article is in the form of a sheet.

12. A method according to any preceding claim, **characterized in that** the article is cooled through said upper temperature range by directing heated air onto at least one surface of the article.

13. A process of producing a heat treatable aluminum alloy sheet article in T4 or T4P temper, which comprises direct chill or continuously casting an alloy to form a casting, subjecting the casting to homogenizing above the solvus temperature of the alloy to dissolve soluble particles present in the casting, hot- and/or cold-rolling the casting to form a sheet article of final gauge, and subjecting the sheet article to solution heat treatment and quenching, **characterized in that** said solution heat treatment and quenching is carried out according to the method of any one of claims 1 to 11.

14. A process according to claim 13, **characterized in that** the hot and/or cold rolling of the casting is carried out with an intermediate annealing step.

## Patentansprüche

1. Verfahren zur Erzeugung eines Gegenstands aus einer lösungsgeglühten Aluminiumlegierung, der frei von permanentem thermischen Verzug ist, wobei diese Legierung in der Lage ist, eine Sekundär-Phasen-Ausscheidung während des Abkühlens nur in einem Ausscheidungs-Temperaturbereich zwischen einer oberen kritischen Temperatur im Bereich von 450 bis 400°C, sowie einer unteren kritischen Temperatur im Bereich von 325 bis 300°C, wobei dieses Verfahren umfasst: Das Unterziehen eines aus der gesagten wärmebehandelbaren Aluminiumlegierung erzeugten Gegenstands einer Lösungs-Glühung bei einer Lösungs-Temperatur oberhalb der oberen kritischen Temperatur, um lösliche Ausscheidungen, die in der Legierung vorliegen, aufzulösen, das Abschrecken des Gegenstands durch diesen Ausscheidungs-Temperaturbereich mit einer Flüssigkeit oder einer Gas/Flüssigkeits-Mischung bei einer Abkühlrate zwischen 200°C/sec und 2000°C/sec., um eine Ausscheidung der Sekundär-Phasen-Partikel zu verhindern, und optional eine zusätzliche Abkühlung des Gegenstands auf eine Temperatur unterhalb der unteren kritischen Temperatur, **dadurch gekennzeichnet, dass** der Gegenstand in einem Gas durch einen oberen Temperaturbereich zwischen der Lösungs-Temperatur und der oberen kritischen Temperatur bei einer Abkühlrate innerhalb des Bereichs von 10°C/sec und 200°C/sec abgekühlt wird, um die Erzeugung von thermischen Spannungen, die stark genug sind, um die Streckgrenze der Legierung in dem oberen Temperaturbereich zu übersteigen, zu verhindern.

2. Verfahren gemäß Anspruch 1, **dadurch gekennzeichnet, dass** das Abkühlen des Gegenstands unter die untere kritische Temperatur in Gas durchgeführt wird.

3. Verfahren gemäß Anspruch 1 oder 2, **dadurch gekennzeichnet, dass** das Abkühlen des Gegenstands unter die untere kritische Temperatur bei einer Rate langsamer als das Abkühlen durch den Ausscheidungs-Bereich durchgeführt wird.

4. Verfahren gemäß Anspruch 1, 2 oder 3, **dadurch gekennzeichnet, dass** das Abkühlen des Gegenstands in dem Gas von der Lösungs-Temperatur zu der oberen kritischen Temperatur in einer einzelnen Abkühlzone durchgeführt wird.

5. Verfahren gemäß Anspruch 1, 2 oder 3, **dadurch gekennzeichnet, dass** das Abkühlen des Gegenstands in dem Gas von der Lösungs-Temperatur zu der oberen kritischen Temperatur in einer Vielzahl von Abkühlzonen durchgeführt wird.

6. Verfahren gemäß Anspruch 5, **dadurch gekennzeichnet, dass** die Temperatur des Gases in jeder aufeinander folgenden Abkühlzone stufenweise geringer ist.

7. Verfahren gemäß Anspruch 6, **dadurch gekennzeichnet, dass** die unteren Temperaturen so gewählt sind, dass sie die Abschreckrate in jeder Zone in Abhängigkeit zu einem Anstieg der Streckgrenze der Legierung in jeder Zone stufenweise erhöhen.

8. Verfahren gemäß einem der voranstehenden Ansprüche, **dadurch gekennzeichnet, dass** die Legierung des Blechgegenstands eine Aluminiumlegierung der AA6000-Serie ist.

9. Verfahren gemäß Anspruch 8, **dadurch gekennzeichnet, dass** der Schritt des Abkühlens des Blechgegenstands von der Lösungs-Temperatur zu der oberen kritischen Temperatur bei einer Rate von etwa 20°C/sec durchgeführt wird.

10. Verfahren gemäß Anspruch 8 oder Anspruch 9, **dadurch gekennzeichnet, dass** der Schritt des weiteren Abkühlens des Blechgegenstands von der oberen kritischen Temperatur zu der unteren kritischen Temperatur bei einer Abkühlrate von zwischen 200°C/sec und 450°C/sec durchgeführt wird.

11. Verfahren gemäß einem der voranstehenden Ansprüche, **dadurch gekennzeichnet, dass** der Gegenstand in der Form eines Blechs vorliegt.

12. Verfahren gemäß einem der voranstehenden Ansprüche, **dadurch gekennzeichnet, dass** der Gegenstand durch den oberen Temperaturbereich durch Richten von erhitzter Luft auf zumindest eine Oberfläche des Gegenstands abgekühlt wird.

13. Verfahren zur Erzeugung eines Blechgegenstands aus einer wärmebehandelbaren Aluminiumlegierung im T4 oder T4P-Temperzustand, welches umfasst: das Direkt-Hartgießen oder kontinuierliche Gießen einer Legierung, um einen Gusskörper auszubilden, Unterziehen des Gusskörpers einer Homogenisierung oberhalb der Solvus-Temperatur der Legierung, um lösliche Partikel, die in dem Gusskörper vorliegen, zu lösen, Warmwalzen und/oder Kaltwalzen des Gusskörpers, um einen Blechgegenstand einer abschließenden Dicke auszubilden, und Unterziehen des Blechgegenstands einer Lösungs-Glühbehandlung, sowie Abschrecken, **dadurch gekennzeichnet, dass** die Lösungs-Glühbehandlung und das Abschrecken gemäß dem Verfahren einer der Ansprüche 1 bis 11 durchgeführt wird.

14. Verfahren gemäß Anspruch 13, **dadurch gekennzeichnet, dass** das Warmwalzen und/oder Kaltwalzen des Gusskörpers mit einem Zwischen-Glühschritt durchgeführt wird.

## Revendications

1. Procédé de production d'un article en alliage d'aluminium qui a subi un traitement thermique de mise en solution, exempt de distorsion thermique permanente, ledit alliage étant capable d'une précipitation de phase secondaire au cours du refroidissement uniquement dans une plage de température de précipitation comprise entre une température supérieure critique dans là plage de 450°C à 400°C et une température inférieure critique dans la plage de 325°C à 300°C, ledit procédé comprenant le fait de soumettre un article composé dudit alliage d'aluminium pouvant subir un traitement thermique à un traitement thermique de mise en solution à une température de mise en solution supérieure à ladite température supérieure critique afin de dissoudre des précipités solubles présents dans ledit alliage, tremper l'article au travers de ladite plage de température de précipitation grâce à un liquide ou à un mélange gaz/liquide à un taux de refroidissement compris entre 200°C/s et 2 000°C/s afin d'éviter une précipitation desdites particules de phase secondaire, et éventuellement refroidir de manière supplémentaire ledit article à une température inférieure à ladite température inférieure critique, **caractérisé en ce que** ledit article est refroidi dans un gaz au travers d'une plage de température supérieure entre ladite température de mise en solution à ladite température supérieure critique à un taux de refroidissement compris dans la plage s'étendant de 10°C/s à 200°C/s afin d'éviter la production de tension thermique suffisamment forte pour dépasser la limite d'élasticité de l'alliage dans ladite plage de température supérieure.

2. Procédé selon la revendication 1, **caractérisé en ce que** ledit refroidissement dudit article au-dessous de ladite température inférieure critique est effectué dans un gaz.

3. Procédé selon la revendication 1 ou 2, **caractérisé en ce que** ledit refroidissement dudit article au-dessous de ladite température inférieure critique est effectué à un taux inférieur audit refroidissement au travers de ladite plage de précipitation.

4. Procédé selon la revendication 1, 2 ou 3, **caractérisé en ce que** le refroidissement de l'article dans le gaz depuis ladite température de mise en solution jusqu'à la température supérieure critique est effectué dans une seule zone de refroidissement.

5. Procédé selon la revendication 1, 2 ou 3, **caractérisé en ce que** le refroidissement de l'article dans le gaz depuis ladite température de mise en solution jusqu'à la température supérieure critique est effectué dans une pluralité de zones de refroidissement.

6. Procédé selon la revendication 5, **caractérisé en ce que** la température du gaz dans chaque zone successive de refroidissement est diminuée progressivement.

7. Procédé selon la revendication 6, **caractérisé en ce que** les températures inférieures sont sélectionnées afin d'augmenter progressivement le taux de trempe dans chaque zone en proportion d'une augmentation de la limite d'élasticité de l'alliage dans chaque zone.

8. Procédé selon l'une quelconque des revendications précédentes, **caractérisé en ce que** ledit alliage dudit article de tôle est un alliage d'aluminium de la série AA6000.

9. Procédé selon la revendication 8, **caractérisé en ce que** ladite étape de refroidissement dudit article de tôle depuis ladite température de mise en solution jusqu'à ladite température supérieure critique est conduit à un taux d'approximativement 20°C/s.

10. Procédé selon la revendication 8 ou 9, **caractérisé en ce que** ladite étape de refroidissement supplémentaire dudit article de tôle depuis la température supérieure critique jusqu'à la température inférieure critique est effectuée à un taux compris entre 200°C/s et 450°C/s.

11. Procédé selon l'une quelconque des revendications précédentes, **caractérisé en ce que** l'article a la forme d'une tôle.

12. Procédé selon l'une quelconque des revendications précédentes, **caractérisé en ce que** l'article est refroidi au travers de ladite plage de température supérieure en dirigeant de l'air chaud sur au moins une surface de l'article.

13. Processus de production d'un article de tôle d'alliage d'aluminium pouvant être traité thermiquement dans une trempe T4 ou T4P, qui comprend un refroidissement direct ou un coulage en continu d'un alliage afin de former une pièce moulée, soumettre la pièce moulée à une homogénéisation au-dessus de la température de solubilité de l'alliage afin de dissoudre les particules solubles présentes dans la pièce moulée, laminer à chaud et/ou à froid la pièce moulée afin de former un article de tôle d'un gabarit final, et soumettre l'article de tôle à un traitement de mise en solution et une trempe, **caractérisé en ce que** ledit traitement de mise en solution et ladite trempe sont effectués selon le procédé de l'une quelconque des revendications 1 à 11.

14. Processus selon la revendication 13, **caractérisé en ce que** ledit laminage à chaud et/ou à froid de la pièce moulé est effectué avec une étape intermédiaire de recuit.
